# EUROPEAN PATENT SPECIFICATION

(11) **EP 0 998 611 B1**
(45) Date of publication and mention of the grant of the patent: **16.02.2005**
(21) Application number: 98936640.6
(22) Date of filing: 21.07.1998
(51) Int. Cl.: E02B 3/06

(54) **A MARINA SYSTEM**
JACHTHAFENANLAGE
SYSTEME DESTINE A UNE MARINA

(30) Priority: 21.07.1997 IE 970530; 21.07.1997 IE 970531
(43) Date of publication of application: 10.05.2000
(73) Proprietor: C O S Holdings Limited, Banagher, County Offaly (IE)
(72) Inventor: LIM, Chong Jin, Nile Lodge, County Galway (IE)
(74) Representative: Gorman, Francis Fergus
(86) International application number: PCT/IE1998/000062
(87) International publication number: WO 1999/005365

(56) References cited:
- FR-A- 2 543 185
- GB-A- 952 186
- GB-A- 2 136 470
- US-A- 4 715 307
- US-A- 4 883 014
- US-A- 5 044 296
- US-A- 5 185 039
- DATABASE WPI Section Ch, Week 8214 Derwent Publications Ltd., London, GB; Class L02, AN 82-27032e XP002082945 & JP 57 034067 A (KAJIMA CORP & SUMITOMO METAL IND LTD), 24 February 1982

## Description

This invention relates to a walkway and more particularly to floating walkways, pontoons, marina systems and the like.

Floating marina systems such as pontoons, walkways and finger pontoons for inland and coastal marina developments are usually made up of three primary structures namely, a structural frame, floatation devices for supporting the structural frame and decking disposed on the structural frame.

The materials from which the components of marina systems are manufactured are critical and should be selected to optimise the durability, practicality, appearance and cost of the marina system.

The decking used in a marina system is usually selected to' optimise the strength, durability, non-slip nature, ease of cleaning and aesthetic appearance of the decking. A one piece reinforced concrete deck has been considered to satisfy the above requirements. However, a number of disadvantages are associated with such one piece reinforced concrete decks. A one piece concrete deck does not facilitate ease of access to facilities and services disposed or housed beneath the decking e.g. for maintenance purposes. In addition, reinforced concrete decking is extremely heavy whilst existing codes of practice for concrete demands a minimum coverage of reinforced concrete on steel reinforcements on the structural frame which further increases the weight of the decking. The additional weight of the reinforced concrete decking enhances the vertical stability characteristics of floating marina systems. However, the significant weight of such reinforced concrete decking also raises the centre of gravity of the one piece reinforced concrete deck which increases the instability of the floating system in wave induced roll.

British Specification No. 2,136,470-A of Moore discloses a paving slab of glass fibre reinforced concrete which comprises a layer of concrete which is typically sandwiched between a pair of glass fibre reinforced layers of a cementitious composition. The paving slab is formed in a mould. A layer of fibre reinforced cementitious composition is initially cast in the mould. A layer of concrete is then cast over the fibre reinforced cementitious composition layer, and optionally this is followed by a final layer of the fibre reinforced cementitious composition. The fibre reinforced layers of cementitious composition may be applied as a pre-mix or a spray, both mechanically or by hand. The material cast into the mould may be subjected to tamping or vibration or rolling to remove air bubbles and to ensure the production of an integrated slab of high strength.

U.S. Patent Specification No. 4,715,307 of Thompson discloses a concrete marine float which forms a deck. A layer of glass fibre reinforced concrete is sprayed into a form over a plasticised polyvinyl chloride mat to a depth of approximately three-quarters of an inch to provide a textured deck surface. While the glass reinforced concrete is still in a semi-liquid or plastic state, a layer of standard aggregate concrete is applied on top of the glass fibre reinforced concrete layer by a pouring process to a predetermined unfinished depth, which typically is of the order of half an inch. Buoyant members are placed over the layer of standard aggregate concrete, which are encased in a shell of glass fibre reinforced concrete.

An object of the invention is to provide a process for the manufacture of a strong and durable reduced weight decking for a marina system which provides a non-slip surface.

According to the invention there is provided a process for the manufacture of a paving slat of glass reinforced concrete, the process comprising the steps of forming a layer of glass fibre reinforced grout and a layer of grout in a mould to form the slat, the layer of glass fibre reinforced grout being sprayed onto the mould, wherein the layer of grout is first formed in the mould by spraying the grout onto the bottom of the mould, a first layer of grout and glass fibre is formed over the layer of grout by spraying, and the first layer of grout and glass fibre is compacted, a second layer of grout and glass fibre is formed over the first layer of grout and glass fibre by spraying, and the second layer of grout and glass fibre is compacted, a final layer of grout and glass fibre is formed over the second layer of grout and glass fibre by spraying, and the final layer of grout and glass fibre is compacted.

Preferably, the glass fibre comprises alkali resistant glass fibre. Suitably, the glass fibre comprises fibres of 12mm to 30mm in length. Preferably, the glass fibre comprises fibres of 25mm in length.

In one embodiment of the invention a reinforcing net is located between the second layer of grout and glass fibre, and the final layer of grout and glass fibre. Advantageously, the reinforcing net is of plastics material, and preferably, is of polypropylene material.

Ideally, the paving slat is in the form of a plank suitable for forming the deck of a walkway, and suitably a plurality of slats is formed into the deck of the walkway, which preferably is the deck of a marina.

The invention also provides a paving slat manufactured by the process according to the invention as a layered structure, wherein the paving slat comprises a layer of grout, a compacted first layer of grout and glass fibre next to the layer of grout, a compacted second layer of grout and glass fibre next to the first layer of grout and glass fibre, and a compacted final layer of grout and glass fibre next to the second layer of grout and glass fibre.

The invention also provides a walkway comprising a deck formed by a plurality of the paving slats according to the invention arranged parallel to each other.

Glass reinforced concrete is an extremely strong material. No metal reinforcements are required with glass reinforced concrete unlike the reinforced concrete systems of the prior art thereby minimising the weight of the material. Accordingly, the glass reinforced concrete deck of the marina systems, walkways and paving of the invention can be comparatively thin compared with the prior art without compromising durability and strength.

Moreover, glass fibre reinforced concrete is an inherently rough material thereby resulting in an non-slip surface without additional treatments being necessary to achieve a gripping surface.

More particularly, glass reinforced concrete provides a non-slip surface without requiring texturing of the surface to achieve the non-slip characteristics. Accordingly, the non-textured surface of the decking 3 of the invention renders the decking 3 easier to clean than with textured systems of the prior art.

In addition, the colour of the glass fibre reinforced concrete decking can be selected during manufacture according to individual requirements.

An embodiment of the invention will now be described, by way of example only, having regard to the accompanying drawings in which:
Fig. 1 is a perspective view of a marina system in accordance with the invention;
Fig. 2 is a top plan view of a pontoon of a marina system in accordance with the invention;
Fig. 3 is a side elevation of the pontoon of Fig. 2;
Fig. 4 is a partial cross-section along the line III-III of Fig. 2;
Fig. 5 is a top plan view of the support frame of the pontoon of Fig. 2;
Fig. 6 is an end elevation of the support frame of Fig. 5;
Fig. 7 is a transverse cross-section along the line VI-VI of Fig. 5;
Fig. 8 is a transverse cross-section along the line VII-VII of Fig. 5;
Fig. 9 is a side elevation of the support frame of Fig. 5;
Fig. 10 is a longitudinal cross-section along the line IX-IX of Fig. 5;
Fig. 11 is a top plan view of an individual decking plank;
Fig. 12 is a side elevation of the decking plank of Fig. 11;
Fig. 13 is a transverse cross-section along the line XIII-XIII of Fig. 11;
Fig. 14 is a top plan view of the floatation tank of the pontoon of the marina system of the invention;
Fig. 15 is an end elevation of the floatation tank of Fig. 14, and
Fig. 16 is a side elevation of the floatation tank.

As shown in the drawings, a typical marina system in accordance with the invention is made up of a series of linked pontoons or walkways 1. Each pontoon 1 is made up of a support frame 2 having decking 3 mounted thereon. The support frame 2 is provided with an outer skin-like fender 4 typically of timber.

The support frame 2 is substantially rectangular in shape and is made up of a first end member 5, a second end member 6, a first side wall 7 and a second side wall 8, all of which are provided with an outer fender 4.

The decking 3 is made up of individual parallel transverse slats, namely planks 9 disposed between the first and second side walls 7,8 of the support frame 2 as shall be explained more fully below.

The support frame 2 together with the decking 3 is mounted on a series of floatation tanks 10 attached to the underside of the support frame 2.

The floatation tanks 10 are substantially box-like in shape and are made up of a rear side wall 11, a front side wall 12, a base wall 13, a top wall 14, a first side wall 15 and a second side wall 16.

The floatation tanks 10 are attached to the underside of the support frame 2 by floatation holders 32 which extend downwards from the support frame 2 as shall be explained more fully below.

Figs. 5 to 10 show various views of the support frame 2 with the decking 3 removed for clarity. As shown in the drawings, the support frame 2 is provided with four elongate ribs 17 which extend parallel to the central longitudinal axis of the support frame 2 between the first and second ends 5,6 parallel to the first and second sides 7,8 of the support frame 2.

The ribs 17 are supported at either end by the first and second end members 5,6 and are each made up of a gusset portion 18 and a channel portion 19. The elongate ribs 17 project upwards into the body of the support frame 2.

As shown in Fig. 8, the first and second side walls 7,8 of the support frame 2 are contoured to define side flanges 20,21 respectively shaped to in turn define inwardly oriented grooves 41. The grooves 41 therefore face each other across the support frame 2.

The ribs 17 are disposed such that the channel portion 19 of the two ribs 17 most adjacent to each side 7,8 of the support frame 2 are disposed to face the groove 41 of the respective side flange 20,21.

The ribs 17 and the side flanges 20,21 together with the respective channel portions 19 and grooves 41 define two side channels 22,23 adjacent the side flanges 20,21 respectively and two intermediate channels 24,25 either side of a centre channel 26 disposed along the central longitudinal axis of the support frame 2.

The support frame 2 is further provided with an end flange 31 similar to the side flanges 20,21 shown in Fig. 7 which also defines an end groove 42 for receiving the support frame 2.

The channels 22,23,24,25 can serve as conduits as required through which pipelines etc. conveying services can be passed.

A pipeline 27 is disposed within the channel 22 and serves to house necessary services such as plumbing and electricity along the length of the marina system of the invention.

Screw holes 28 are disposed along the first and second side walls 7,8 of the support frame 2 for attaching the fenders 4 to the support frame 2.

As shown in Fig. 7, the support frame 2 is further provided with stiffeners 29 and stiffening plates 30 disposed and spaced apart along the length of the elongate ribs 17. The stiffeners and plates 29,30 respectively serve to reinforce the support frame structure 2.

The float holders 32 extend downwards from the support frame 2 i.e. in a direction opposite to the decking 3 to support the floatation tanks 10.

Figs. 11 to 13 show enlarged views of an individual plank 9 of the decking 3. As shown in the drawings, the plank 9 is rectangular in shape and is provided with screw holes 28 disposed along the plank 9 for attaching the plank 9 to the support frame 2. The screw holes 28 are located on the plank 9 to correspond to the location of the ribs 17 such that screws inserted through the screw holes 28 extend into the ribs 17.

Internally, each plank screw hole 28 is made up of plastic tubing 33 disposed transversely within the plank 9 and a rebate 34 adjacent the surface of the plank 9 for receiving a self tapping screw.

Each plank 9 contains a transverse sheet of polypropylene netting 35 disposed parallel to the top and bottom faces of the plank 9 such that the propylene netting is encased by the material of the plank 9 and is concealed within the plank 9.

Figs. 14 to 16 show enlarged views of a floatation tank 10 of the pontoon 1. The floatation tank 10 is substantially box-like in shape and is made up of a rear side wall 11, a front side wall 12, a base 13, a top wall 14, a first side wall 15 and a second side wall 16 as previously described. An upwardly extending threaded fixing bar 36 is disposed adjacent each corner at the top face 14 of the floatation tank 10. The threaded fixing bar 36 is provided with a base plate 39 disposed within the top face 14 on which the floatation tank 10 is supported. Each wall of the material of the floatation tank 10 is reinforced with an inner aeroboard block to aid flotation 37. The aeroboard block 37 is shaped to define a corner recess 38 in which the base plate 39 is disposed adjacent each corner of the floatation tank 10. In addition, a polypropylene net 35 is disposed adjacent each threaded fixing bar 36 to reinforce the walls 11,12,13,14,15 and 16 of the floatation tank 10.

The planks 9 used in the decking 3 of the marina system in accordance with the invention facilitate easy access to the support frame 2 and the pipeline 27 disposed within the support frame 2 by simple removal as required of individual planks 9 thereby providing easy access to the support frame 2.

The planks 9 of the marina system of the invention are manufactured from glass fibre reinforced concrete.

### Glass Fibre Reinforced Concrete

The walkways, pontoons, and marina systems of the invention are made of glass fibre reinforced concrete. Alkali resistant (AR) glass fibre is particularly preferred in the manufacture of the glass fibre reinforced concrete planks according to the invention. AR resistant glass fibre is advantageous as it is more resistant to attack from the alkali normally present in cement compared with normal glass fibre. Moreover, AR glass fibre has particularly good non-combustibility characteristics, is corrosion resistant, and has a high tensile strength similar to piano wire. Suitable glass fibres are available from NEG while a particularly preferred AR glass fibre reinforced concrete is also available from NEG.

Further advantages associated with glass fibre reinforced concrete are:
Flexibility of design;
High impact strength;
High bending strength;
A high toughness and cracking resistivity;
Light weight due to thin section, and
Non-combustibility.

The fibre lengths of the glass fibre can range from approximately 12mm to 30mm. A glass fibre length of 25mm is particularly preferred as it has been found that such a fibre length provides optimum length from both a workability and structural point of view and provides a glass reinforced concrete product having the desired structural integrity. Shorter glass fibres have been found to render the concrete mix more workable. However, excessively short glass fibre lengths have been found to slip excessively in the concrete.

The percentage weight of glass fibre used in the concrete is varied according to the strength and workability required of the concrete. Typically, a glass fibre is used in a percentage rate of 0.5% to 5% by weight of the concrete. Excessively low percentages of fibre offer minimum strength advantage over plain concrete with the strength of glass fibre reinforced concrete increasing as the percentage of glass fibre is increased.

However, excessively high amounts of glass fibre have been found to reduce the workability of the glass fibre reinforced concrete excessively.

In an alternative embodiment of the invention, the glass fibre used in the concrete can be in the form of elongate rods or rebars inserted in the concrete during moulding of the planks 9. An advantage to using elongate rods of glass fibre is that the rods help to resist breakages thereby reinforcing the planks 9 and obviating the requirement of the netting 35. A suitable rebar for the marina system of the present invention is a 6mm diameter glass fibre reinforced polymer rebar. In the present embodiment of the invention the netting 35 could be replaced by three such rebars spaced apart within the concrete of the planks 9. Suitable glass fibre reinforced polymer rods are available from Hughes Brothers Incorporated, Nebraska, United States.

Dye is added in the glass reinforced concrete according to the colour required of the final plank 9. A wide range of colours may be utilized.

Any kind of concrete dye may be used in the manufacture of the glass fibre reinforced concrete. Suitable dyes are available from Harcros Pigments Limited.

An example of a glass reinforced concrete mixture suitable for use in the manufacture of the plank 9 is given by way of the following non-limiting example:

### EXAMPLE 1:

| MATERIAL | WEIGHT |
|---|---|
| Ordinary Portland | |
| Cement (OPC) | 50Kg |
| Sand | 50Kg |
| Water | 17.5Kg |
| Super Plasticiser | .02Kg |
| AR glassfibre | 6.2Kg |
| Colour dye | As desired |

The glass reinforced concrete mix was mixed as follows:

### Equipment Required:

A high shear mixer; a power sprayer which consisted of a spray gun connected to an air compressor which was fed by a grout hopper; a chopper for dosing glass fibre; and suitably shaped moulds.

### Method:

Before production was begun the required moulds were cleaned, oiled and left ready for spraying.

The required amounts of water and additive were released into the mixer and the mixer was started at a slow speed.

The sand and cement were added to the mixing bucket of the mixer. The sand was added first, and the mixer was turned up to a high speed. The cement was then added. The constituents were left to mix for approximately 1 minute.

At this stage dye was added to the mix if required and left to mix for a further 1 minute. The resulting grout was now ready for spraying.

Before the grout is placed in the power sprayer, the sprayer is washed out thoroughly with clean water. The nozzle is lubricated with washing-up-liquid and placed on the sprayer. The hose is then connected to the nozzle and the spray gun is connected to the hose and air pipes.

The compressor is started and all air pressures are checked.

The glass fibre is typically in the form of a roll which is fed into the gun as will be appreciated by those skilled in the art. The gun is in communication with a chopper to control spraying of glass fibre portions chopped from the roll through the gun.

The grout was then charged into the hopper.

The moulds required to be sprayed were put into position. First of all a 3mm layer of grout was sprayed onto the bottom of the moulds, a layer of grout and fibre was then sprayed over the first layer using the gun. This layer was then compacted with the use of a roller. Another layer of grout and fibre was then sprayed and this layer was compacted as before. A strip of reinforcing/polypropylene netting was placed on top of this layer. The final layer of grout and fibre was then applied. This layer was compacted as before and then levelled and finished off using a steel trowel.

The moulds were then stacked and new moulds put into position for spraying. When all the moulds required were filled and stacked, the stacks were covered and left to set. The moulds were stripped the following day and got ready for respraying.

The floatation tanks 10 used in the marina system of the invention are typically manufactured from polystyrene aeroboard encased in concrete. An advantage of such floatation tank material is the high degree of durability and stability enjoyed by the floatation tanks 10. The floatation tanks 10 of the marina system of the invention are manufactured from a concrete having comparatively short glass fibre strands contained within the concrete.

The purpose of the concrete casing of the floatation tanks is to protect the encased polystyrene material from damage. The concrete casing of the floatation tanks is not required to provide structural support unlike the glass fibre reinforced concrete of the planks 9. Accordingly, the structural strength requirements of the concrete of the floatation tanks are not as rigorous as those of the planks 9.

A typical floatation tank concrete mix was as follows:

### EXAMPLE 2:

| MATERIAL | WEIGHT |
|---|---|
| Cement OPC | 225Kg |
| Sand | 700Kg |
| Water | 150Kg |
| Super Plasticiser | 7Ltrs |
| AR 12mm Chopped Glassfibre | 4.5Kg |
| Aeroboard | |

The percentage rate of glass fibre utilised in the construction of the glass fibre reinforced concrete of the floatation tank is less than that required for the planks 9 as described in relation to Example 1. More particularly, a lower percentage is required as the skin of the floatation tank is non-structural while the purpose of the glass fibre in the skin is to reduce cracking of the skin. Accordingly, the percentage rate of fibre used in the manufacture of the skin was typically around 0.5%.

The length of fibre utilised in the production of the glass fibre reinforced concrete floatation tank was typically 12mm.

The floatation tank mixture was formed into a floatation tank as follows:
A floatation tank mould was employed which consisted of two main parts - an upper steel shutter and concrete base of the following fixed dimensions: 3000 x 1500 x 150mm. The steel shutter was interchangeable and could be increased or decreased in length or width depending on production requirements.

When production was due to begin, the mould was cleaned oiled and squared. The floatation tank was cast upside-down. Four holes were predrilled in the slab to receive threaded bars which were anchored in the blocks using reinforced netting. The threaded bars were used to connect the walkways to the floatation tanks.

The aeroboard 37 was then chamfered and four holes cut out of each corner with the aid of a template.

The glass fibre reinforced concrete mix was transported from the mixer to the moulds.

The base was poured first and levelled off to a depth of about 20mm. The aeroboard 37 was then placed in the mould and spacers fixed around the sides. Clamps were placed across the top of the mould to hold the aeroboard down during pouring. The sides were then filled, the spacers were removed and the sides topped off with concrete. The sides were compacted lightly. After an initial set the clamps were lifted and the top was screeded to the required depth. The edge was chamfered off with a bull-nose trowel. The mould was then covered.

The following day the moulds were stripped. After a few days drying time the floatation tanks were turned, right-side-up fitted with nuts and washers. The floatation tanks were then stacked and ready for delivery.

In use, a marina system as shown in Fig. 1 is assembled from pontoons 1 as previously described. A typical marina system is provided with a primary walkway or pontoon 1 and secondary walkways or pontoons 43 attached to the primary pontoon 1. Each pontoon 43 is provided with floatation tanks 10 also as previously described. Mooring mountings 44 are disposed on the support frame 2 for mooring boats etc.

The pontoons 1,43 are connected by connecting frames 45 to secure the secondary pontoons 43 to the primary pontoon 1 at the support frame 2 of the primary pontoon 1 and secondary pontoon 43.

The primary pontoon 1 and the secondary pontoons 43 are provided with upstanding service posts 46 so that boats etc attach to moorings 44 can receive electrical power, water and other services from the service posts 46. The service posts 46 are mounted on the planks 9 and are in communication with the service pipe 27 disposed beneath the planks 9 as previously described.

The marina system of the invention is held in place by mounting posts 47 inserted in the sea, river or lake bed. The primary pontoon 1 is attached to the mounting post 47 by brackets 48 which enjoy a sliding relationship with the upstanding mounting posts 47 so that the marina system of the invention can ride upwards and downwards on the mounting posts 47 as the water level rises and decreases.

Typically, the glass fibre reinforced concrete decking is manufactured in plank form with a standard plank width of 300mm. The plank 9 can be attached to the support frame 2 with stainless steel self tapping screws through the holes 28 cast in the plank.

The use of the plastics tubing 33 in the screw holes 28 avoids stresses experienced the support frame 2 in use from being transmitted to the plank 9.

In addition, the use of separate plank 9 facilitates replacement of individual plank 9 should damage occur.

The use of a polypropylene net in the glass fibre reinforced concrete material used in the marina system of the invention enhances the structural integrity of the glass fibre reinforced concrete and prevents complete separation of a plank 9 should a plank 9 become fractured. However, where glass fibre reinforced polymer rebars are employed no netting is required.

The support frame 2 is manufactured from galvanised steel or any other suitable material. An advantage of galvanised steel is that galvanised steel provides flexibility to the support frame 2 which is advantageous during the twisting load experienced by a support frame on waves etc. Galvanised steel is also highly compatible with glass fibre reinforced concrete decking 3.

The threaded fixing bar 36 and backing plate 39 are suitably manufactured from stainless steel bolts cast into the glass fibre reinforced concrete.

The marina system of the invention is stable under off-shore weather conditions and is suitable for use in the assembly of elongate finger piers.

The colour adaptability of the marina system of the invention ensures that a wide variety of colours can be used or blended in the manufacture of marina systems to render the marina system compatible with local and environmental surroundings. Alternatively, the marina system can be coloured to reflect or portray corporate or club colours etc.

## Claims

1. A process for the manufacture of a paving slat of glass reinforced concrete, the process comprising the steps of forming a layer of glass fibre reinforced grout and a layer of grout in a mould to form the slat, the layer of glass fibre reinforced grout being sprayed onto the mould, **characterised in that** the layer of grout is first formed in the mould by spraying the grout onto the bottom of the mould, a first layer of grout and glass fibre is formed over the layer of grout by spraying, and the first layer of grout and glass fibre is compacted, a second layer of grout and glass fibre is formed over the first layer of grout and glass fibre by spraying, and the second layer of grout and glass fibre is compacted, a final layer of grout and glass fibre is formed over the second layer of grout and glass fibre by spraying, and the final layer of grout and glass fibre is compacted.

2. A process as claimed in Claim 1 **characterised in that** the glass fibre is alkali resistant glass fibre.

3. A process as claimed in Claim 1 or 2 **characterised in that** the glass fibre comprises fibres of length in the range of 12mm to 30mm.

4. A process as claimed in Claim 3 **characterised in that** the fibres of the glass fibre are of length of 25mm.

5. A process as claimed in any preceding claim **characterised in that** a reinforcing net is placed on top of the second layer of grout and glass fibre prior to forming the final layer of grout and glass fibre.

6. A process as claimed in Claim 5 **characterised in that** the reinforcing net is of plastics material.

7. A process as claimed in Claim 6 **characterised in that** the plastics material of the reinforcing net is polypropylene material.

8. A process as claimed in any preceding claim **characterised in that** the paving slat is in the form of a plank suitable for forming the deck of a walkway.

9. A process as claimed in Claim 8 **characterised in that** the plank is suitable for forming the deck of a marina.

10. A paving slat manufactured by the process as claimed in any preceding claim as a layered structure, **characterised in that** the paving slat comprises a layer of grout, a compacted first layer of grout and glass fibre next to the layer of grout, a compacted second layer of grout and glass fibre next to the first layer of grout and glass fibre, and a compacted final layer of grout and glass fibre next to the second layer of grout and glass fibre.

11. A walkway comprising a deck formed by a plurality of paving slats as claimed in Claim 10 arranged parallel to each other.

12. A marina comprising the walkway as claimed in Claim 11.

## Patentansprüche

1. Verfahren zur Herstellung einer Belaglatte aus glasverstärktem Beton, das Verfahren umfassend die Schritte des Bildens einer Schicht aus glasfaserverstärktem Mörtel und einer Mörtelschicht in einer Form zum Ausbilden der Latte, wobei die Schicht aus glasfaserverstärktem Mörtel auf die Form gesprüht wird, **dadurch gekennzeichnet, dass** die Mörtelschicht zuerst in der Form ausgebildet wird, indem der Mörtel auf den Boden der Form gesprüht wird, eine erste Schicht aus Mörtel und Glasfaser über der Mörtelschicht durch Sprühen ausgebildet wird und die erste Schicht aus Mörtel und Glasfaser kompaktiert wird, eine zweite Schicht aus Mörtel und Glasfaser über der ersten Schicht aus Mörtel und Glasfaser durch Sprühen ausgebildet wird und die zweite Schicht aus Mörtel und Glasfaser kompaktiert wird, eine letzte Schicht aus Mörtel und Glasfaser über der zweiten Schicht aus Mörtel und Glasfaser durch Sprühen ausgebildet wird und die letzte Schicht aus Mörtel und Glasfaser kompaktiert wird.

2. Verfahren nach Anspruch 1, **dadurch gekennzeichnet, dass** die Glasfaser eine alkaliresistente Glasfaser ist.

3. Verfahren nach Anspruch 1 oder 2, **dadurch gekennzeichnet, dass** die Glasfaser Fasern mit einer Länge im Bereich zwischen 12 mm und 30 mm umfasst.

4. Verfahren nach Anspruch 3, **dadurch gekennzeichnet, dass** die Fasern der Glasfaser eine Länge von 25 mm aufweisen.

5. Verfahren nach einem der vorhergehenden Ansprüche, **dadurch gekennzeichnet, dass** ein Verstärkungsnetz auf der zweiten Schicht aus Mörtel und Glasfaser vor dem Ausbilden der letzten Schicht aus Mörtel und Glasfaser platziert wird.

6. Verfahren nach Anspruch 5, **dadurch gekennzeichnet, dass** das Verstärkungsnetz aus einem Plastikmaterial besteht.

7. Verfahren nach Anspruch 6, **dadurch gekennzeichnet, dass** das Plastikmaterial des Verstärkungsnetzes ein Polypropylenmaterial ist.

8. Verfahren nach einem der vorhergehenden Ansprüche, **dadurch gekennzeichnet, dass** die Belaglatte die Gestalt einer Planke aufweist, welche geeignet ist, das Deck eines Gehwegs zu bilden.

9. Verfahren nach Anspruch 8, **dadurch gekennzeichnet, dass** die Planke geeignet ist, das Deck eines Yachthafens zu bilden.

10. Belaglatte hergestellt als eine Schichtstruktur nach dem Verfahren gemäß einem der vorgehenden Ansprüche, **dadurch gekennzeichnet, dass** die Belaglatte eine Mörtelschicht umfasst, eine kompaktierte erste Schicht aus Mörtel und Glasfaser angrenzend an die Mörtelschicht, eine kompaktierte zweite Schicht aus Mörtel und Glasfaser angrenzend an die erste Schicht aus Mörtel und Glasfaser und eine kompaktierte letzte Schicht aus Mörtel und Glasfaser angrenzend an die zweite Schicht aus Mörtel und Glasfaser.

11. Gehweg umfassend ein Deck, das aus einer Vielzahl von Belaglatten nach Anspruch 10 gebildet ist, die parallel zueinander ausgerichtet sind.

12. Yachthafen umfassend den Gehweg nach Anspruch 11.

## Revendications

1. Processus pour la fabrication d'une dalle de revêtement de sol en béton renforcé de verre, le processus comprenant les étapes consistant à former une couche de mortier renforcé de fibres de verre et une couche de mortier dans un moule afin de former la dalle, la couche de mortier renforcé de fibres de verre étant pulvérisée dans le moule, **caractérisé en ce que** la couche de mortier est tout d'abord formée dans le moule en pulvérisant le mortier au fond du moule, une première couche de mortier et de fibres de verre est formée par-dessus la couche de mortier par pulvérisation, et la première couche de mortier et de fibres de verre est compactée, une seconde couche de mortier et de fibres de verre est formée par-dessus la première couche de mortier et de fibres de verre par pulvérisation, et la seconde couche de mortier et de fibres de verre est compactée, une couche finale de mortier et de fibres de verre est formée par-dessus la seconde couche de mortier et de fibres de verre par pulvérisation, et la couche finale de mortier et de fibres de verre est compactée.

2. Processus selon la revendication 1, **caractérisé en ce que** les fibres de verre sont des fibres de verre résistant aux alcalis.

3. Processus selon la revendication 1 ou 2, **caractérisé en ce que** les fibres de verre comprennent des fibres ayant une longueur de l'ordre de 12 mm à 30 mm.

4. Processus selon la revendication 3, **caractérisé en ce que** les fibres des fibres de verre possèdent une longueur de 25 mm.

5. Processus selon l'une quelconque des revendications précédentes, **caractérisé en ce qu'**un filet de renforcement est placé au sommet de la seconde couche de mortier et de fibres de verre avant de former la couche finale de mortier et de fibres de verre.

6. Processus selon la revendication 5, **caractérisé en ce que** le filet de renforcement est en matériau plastique.

7. Processus selon la revendication 6, **caractérisé en ce que** le matériau plastique du filet de renforcement est un matériau en polypropylène.

8. Processus selon l'une quelconque des revendications précédentes, **caractérisé en ce que** la dalle de revêtement de sol est sous la forme d'un plateau convenant pour former le pont d'une passerelle.

9. Processus selon la revendication 8, **caractérisé en ce que** le plateau convient pour former le pont d'une marina.

10. Dalle de revêtement de sol fabriquée par le processus selon l'une quelconque des revendications précédentes comme une structure stratifiée, **caractérisée en ce que** la dalle de revêtement de sol comprend une couche de mortier, une première couche compactée de mortier et de fibres de verre proche de la couche de mortier, une seconde couche compactée de mortier et de fibres de verre proche de la première couche de mortier et de fibres de verre, et une couche finale compactée de mortier et de fibres de verre proche de la seconde couche de mortier et de fibres de verre.

11. Passerelle comprenant un pont formé d'une pluralité de dalles de revêtement de sol selon la revendication 10, agencées parallèlement les unes aux autres.

12. Marina comprenant la passerelle selon la revendication 11.
